



US007575643B2

(12) **United States Patent**  
**Ebihara et al.**

(10) **Patent No.:** **US 7,575,643 B2**  
(45) **Date of Patent:** **Aug. 18, 2009**

(54) **CARBURIZATION TREATMENT METHOD**

(75) Inventors: **Hisashi Ebihara**, Tokyo (JP); **Jun Takahashi**, Tokyo (JP); **Fumitaka Abukawa**, Tokyo (JP); **Keiji Yokose**, Tokyo (JP); **Hidetoshi Juryozawa**, Tokyo (JP)

(73) Assignee: **Dowa Mining Co., Ltd.**, Tokyo (JP)

(\*) Notice: Subject to any disclaimer, the term of this patent is extended or adjusted under 35 U.S.C. 154(b) by 0 days.

(21) Appl. No.: **10/107,206**

(22) Filed: **Mar. 28, 2002**

(65) **Prior Publication Data**

US 2002/0179186 A1 Dec. 5, 2002

(30) **Foreign Application Priority Data**

Jun. 5, 2001 (JP) ..... 2001-169636

(51) **Int. Cl.**  
**C22C 8/22** (2006.01)  
**C23C 8/00** (2006.01)

(52) **U.S. Cl.** ..... **148/223**; 148/235

(58) **Field of Classification Search** ..... 148/235,  
148/223

See application file for complete search history.

(56) **References Cited**

U.S. PATENT DOCUMENTS

4,386,973 A \* 6/1983 Kawka et al. ..... 148/223  
5,827,375 A \* 10/1998 Barbour ..... 148/225

OTHER PUBLICATIONS

"Heat treating in vacuum furnaces and auxiliary equipment", ASM Handbook, Heat Treating, vol. 4, 1991, sections "Introduction" and "Comparison of vacuum and atmosphere furnace processing."

\* cited by examiner

Primary Examiner—Sikyin Ip

(74) Attorney, Agent, or Firm—Pillsbury Winthrop Shaw Pittman, LLP

(57) **ABSTRACT**

The invention provides a carburization treatment method in which the carburization treatment is conducted under a condition where an atmosphere within the furnace is maintained at a high carbon potential which is slightly below a carbon solid solubility. Preferably, the internal pressure within the furnace is kept at 0.1 to 101 kPa, the hydrocarbon gas is one, two or more than two kinds of gases selected from the group consisting of C<sub>3</sub>H<sub>8</sub>, C<sub>3</sub>H<sub>6</sub>, C<sub>4</sub>H<sub>10</sub>, C<sub>2</sub>H<sub>2</sub>, C<sub>2</sub>H<sub>4</sub>, C<sub>2</sub>H<sub>6</sub> and CH<sub>4</sub>, while the oxidative gas is an air, an O<sub>2</sub> gas, or CO<sub>2</sub> gas.

**6 Claims, 4 Drawing Sheets**



**Fig. 1****Fig. 2**

**Fig. 3****Fig. 4**

**Fig. 5****Fig. 6**

**Fig. 7**



## 1

## CARBURIZATION TREATMENT METHOD

## CROSS REFERENCE TO RELATED APPLICATIONS

This application claims priority to Japanese patent application No. 2001-169636, filed Jun. 5, 2001, which is incorporated by reference herein in its entirety.

## BACKGROUND OF THE INVENTION

## 1. Field of the Invention

The present invention relates to carburization treatment methods for carburizing steel material.

## 2. Description of the Related Art

Various methods are known for carburizing steel material, such as a gas carburization method, a vacuum carburization method, and a plasma carburization method, with each having both advantages and disadvantages.

However, one gas carburization method has a disadvantage of the generation of a large amount of  $\text{CO}_2$  gas and a possibility of an explosion. A further problem associated with this method is that intergranular oxidation will occur on the surface of the steel material. On the other hand, another gas carburization method using an endothermic gas makes it necessary to employ a metamorphism furnace, hence suffering from a problem of high equipment cost.

A vacuum carburization method is associated with a problem in that once the carbon concentration on the surface of a steel material is increased to a predetermined solid solubility, a large amount of soot will be undesirably generated. As a result, not only does the carburization equipment need a comparatively long time and a considerably high cost for maintenance, but also such equipment does not have sufficient versatility. Moreover, another problem associated with this method is that it is difficult to perform a carbon potential control in an atmosphere within the furnace, if compared with the above-described gas carburization methods. In addition, a plasma carburization method is said to be low in productivity.

## SUMMARY OF THE INVENTION

Accordingly, it is an object of the present invention to provide improved, new and economical carburization treatment methods which can be effectively used to replace any one of the above-described conventional carburization methods.

In order to achieve the above objects of the present invention, a carburization treatment method according to the present invention is characterized in that the carburization treatment is conducted while maintaining the atmosphere within the furnace at a high carbon potential which is slightly below a carbon solid solubility limit. With the use of this method, it becomes possible to shorten the carburization lead time and to reduce the total energy consumption.

Further, according to the above method of the present invention, the carburization treatment is carried out under a condition where the internal pressure of the furnace has been reduced. With the use of this method, the reduced internal pressure of the furnace makes it possible to stabilize the atmosphere having a high carbon potential. Moreover, since it is possible to prevent the generation of soot, easier maintenance of the furnace can be achieved.

In addition, as another preferred embodiment of the present invention, the internal pressure within the furnace is 0.1 to 101 kPa. In other words, if the internal pressure within the furnace is lower than 0.1 kPa, it is impossible to ensure a

## 2

desired carburization capability. On the other hand, if the internal pressure within the furnace is larger than 101 kPa, since such an internal pressure is generally close to atmospheric pressure, a problem will be caused which is similar to that associated with the above-described conventional gas carburization method.

As a further preferred embodiment of the present invention, an atmosphere having a high carbon potential slightly below the carbon solid solubility is maintained by directly supplying the hydrocarbon gas and/or the oxidative gas into the furnace. With the use of this method of the present invention, since such a method is different from the above-described vacuum carburization method in that at least one of the hydrocarbon gas and the oxidative gas is supplied into the furnace, it becomes possible to control the atmosphere within the furnace, thus making it easy to maintain the atmosphere within the furnace at a high carbon potential which is slightly below the carbon solid solubility. Moreover, since it is possible to dispense with an exhaust gas burning process (which was needed in the above-described conventional gas carburization method),  $\text{CO}_2$  gas generation is prevented so that there is no possibility of an explosion. Further, since it is not necessary to employ a metamorphism furnace, the amount of gas necessary to be used in the carburization treatment can be reduced, thereby rendering the whole process of carburization treatment more economic.

In the above-described method, for use as the hydrocarbon gas it is possible to utilize at least one selected from the group consisting of  $\text{C}_3\text{H}_8$ ,  $\text{C}_3\text{H}_6$ ,  $\text{C}_4\text{H}_{10}$ ,  $\text{C}_2\text{H}_2$ ,  $\text{C}_2\text{H}_4$ ,  $\text{C}_2\text{H}_6$ ,  $\text{CH}_4$ . On the other hand, for use as the oxidative gas it is possible to utilize air, an  $\text{O}_2$  gas, or  $\text{CO}_2$  gas.

Further, in the above-described method, the amount of at least one of the hydrocarbon gas and the oxidative gas being supplied to the furnace for maintaining an atmosphere having a high carbon potential slightly below the carbon solid solubility, is controlled by carrying out at least one of the following measurements which include: measurement of  $\text{CO}$  gas partial pressure, measurement of  $\text{CO}$  gas concentration, measurement of  $\text{CO}_2$  gas partial pressure, measurement of  $\text{CO}_2$  gas concentration, measurement of  $\text{O}_2$  gas partial pressure, measurement of  $\text{O}_2$  gas concentration, measurement of  $\text{H}_2$  gas partial pressure, measurement of  $\text{H}_2$  gas concentration, measurement of  $\text{CH}_4$  gas partial pressure, measurement of  $\text{CH}_4$  gas concentration, measurement of  $\text{H}_2\text{O}$  partial pressure, measurement of  $\text{H}_2\text{O}$  concentration, and measurement of dew point, all within the furnace.

## BRIEF DESCRIPTION OF THE DRAWINGS

FIG. 1 is an explanatory view showing a carburization furnace suitable for carrying out the carburization treatment method according to the present invention.

FIG. 2 is a plan view showing the structure of a carburization quenching apparatus suitable for carrying out the carburization treatment method according to the present invention.

FIG. 3 is a graph showing an average carbon concentration distribution of a steel material treated in Example 1.

FIG. 4 is a photograph showing the surface organization of the steel material treated in Example 1.

FIG. 5 is a graph showing an average carbon concentration distribution of a steel material treated in Example 2.

FIG. 6 is a photograph showing the surface organization of the steel material treated in Example 2.

FIG. 7 is also a photograph but showing the crystal particles of the steel material treated in Example 2.

## DESCRIPTION OF THE PREFERRED EMBODIMENTS

Referring to FIG. 1, reference numeral 1 represents a furnace casing, reference numeral 2 represents a thermally insulating material, reference numeral 3 represents an atmosphere stirring fan, reference numeral 4 represents a heater, reference numeral 5 represents a thermal couple for measuring an internal temperature within the furnace, reference numeral 6 represents a pressure gauge for use in controlling and reducing an internal pressure within the furnace, reference numeral 7 represents a sampling device for sampling an atmosphere within the furnace, reference numeral 8 represents an analyzer for analyzing an atmosphere within the furnace, such an analyzer may be a CO gas partial pressure gauge or a CO gas concentration meter. Reference numeral 9 represents an analyzer for analyzing an atmosphere within the furnace, but such an analyzer may be a CO<sub>2</sub> gas partial pressure gauge or a CO<sub>2</sub> gas concentration meter. Reference numeral 30 represents a further analyzer for analyzing an atmosphere within the furnace, such an analyzer may be an O<sub>2</sub> gas partial pressure gauge or an O<sub>2</sub> gas concentration meter. Reference numeral 10 represents a mass flow controller provided in connection with a hydrocarbon gas supply unit 10a for controlling an amount of hydrocarbon gas to be supplied to the furnace. Reference numeral 11 represents another mass flow controller provided in connection with an oxidative gas supply unit 11a for controlling an amount of an oxidative gas to be supplied to the furnace. Reference numeral 12 represents a vacuum pump for reducing an internal pressure within the furnace. Reference numeral 13 represents a carbon potential computing device, reference numeral 14 represents a regulation device for sending regulation signals to the mass flow controllers 10 and 11 in accordance with the computed values fed from the carbon potential computing device 13. Here, the thermally insulating material 2 is preferably made of a ceramic fiber having a low heat radiation and a low heat accumulation.

With regard to the aforementioned carburization furnace having the above-described construction, the pressure reduction adjustment within the furnace can be carried out by controlling the discharge of an atmosphere from the furnace, by virtue of the pressure gauge 6 and the vacuum pump 12. Further, the carbon potential of an atmosphere within the furnace may be controlled in a manner described as follows, so that it is possible to maintain a high carbon potential which is slightly below a carbon solid solubility. At this time, the analysis values fed from the internal atmosphere analyzers 8, 9 and 30 are introduced into the carbon potential computing device 13. Then, the adjustment gauge 14, in accordance with the computed values provided by the carbon potential computing device 13, operates to send an adjustment signal to the mass flow controller 10 (for controlling the hydrocarbon gas supply amount) as well as to the mass flow controller 11 (for controlling the oxidative gas supply amount). In this way, it is possible to adjust an amount of at least one of the hydrocarbon gas and the oxidative gas being supplied into the furnace, thereby effectively controlling the carbon potential of an atmosphere within the furnace.

The control of an amount of the hydrocarbon gas and/or the oxidative gas being supplied into the furnace may be effected by measuring the partial pressure of at least one of various kinds of gases forming an atmosphere within the furnace. However, it is also possible to perform the same control by measuring the concentration of at least one of various kinds of gases forming the atmosphere within the furnace. For example, it is possible to measure the partial pressure or the

concentration of at least one of CO gas, CO<sub>2</sub> gas, O<sub>2</sub> gas, H<sub>2</sub> gas and CH<sub>4</sub> gas (together forming an atmosphere within the furnace), by utilizing various partial pressure gauges (CO gas partial pressure gauge, CO<sub>2</sub> gas partial pressure gauge, O<sub>2</sub> gas partial pressure gauge, H<sub>2</sub> gas partial pressure gas and CH<sub>4</sub> gas partial pressure gas) or various concentration meters (CO gas concentration meter, CO<sub>2</sub> gas concentration meter, O<sub>2</sub> gas concentration meter, H<sub>2</sub> gas concentration meter and CH<sub>4</sub> gas concentration meter), thereby effecting correct control of the supply amount of the hydrocarbon gas and/or the oxidative gas when being supplied into the furnace.

Furthermore, it is possible to control an amount of the hydrocarbon gas and/or the oxidative gas being supplied into the furnace, by measuring the partial pressure of H<sub>2</sub>O or the concentration of H<sub>2</sub>O within the furnace, or by measuring the dew point of an atmosphere gas within the furnace using a dew point hygrometer.

In this way, with the use of the various methods as described in the above, it is possible to correctly control an amount of the hydrocarbon gas and/or the oxidative gas being supplied into the furnace, thereby making it possible to keep an atmosphere within the furnace at a high carbon potential which is slightly below the carbon solid solubility.

Referring to FIG. 2, reference numeral 15 represents an inlet door, reference number 16 represents a transportation room, reference numeral 17 represents a carburization room, reference numeral 18 represents a gas cooling room, reference numeral 19 represents an oil quenching room, reference numeral 20 represents an outlet door, while reference numerals 21a, 21b and 21c all represent partition doors. Here, the carburization room 17 is identical to the carburization room in the carburization furnace shown in FIG. 1.

An initial state of the carburization quenching apparatus will be described as follows. Namely, the inlet door 15, the outlet door 20 and the partition doors 21a, 21b and 21c are all closed. The carburization room 17 is heated to a quenching temperature and then kept at this temperature, while the pressure within the carburization room is controlled at 0.1 kPa or lower. Similarly, the pressure within the quenching room 19 is also kept at 0.1 kPa or lower, while the quenching oil within the quenching room 19 is heated to a temperature suitable for steel material quenching treatment. At this time, the transportation room 16 is under atmospheric pressure.

Starting from the above-described initial state, at first, the inlet door 15 is opened so that steel material is introduced into the transportation room 16. Then, the inlet door 15 is closed and the pressure within the transportation room 16 is reduced to 0.1 kPa or lower. Subsequently, the partition door 21a located between the transportation room 16 and the carburization room 17 is opened so that the steel material is moved to the carburization room 17. Then, the partition wall 21 is closed. On the other hand, although not shown in the drawings, an apparatus for transporting the steel material may be a chain device (for use in the transportation room 16 as well as in the oil quenching room 19 and driven by a motor, and may also be a roller hearth for use in the carburization room 17).

Then, after the partition door 21a is closed, the pressure within the carburization room 17 recovers to a predetermined pressure such as 100 kPa by virtue of N<sub>2</sub> gas, while the temperature within the carburization room is elevated to the carburization temperature. Subsequently, after the carburization room has been kept at the carburization temperature for 30 minutes, N<sub>2</sub> gas is discharged from the carburization room 17, so that the pressure within the carburization room 17 is reduced to 0.1 kPa or lower.

Afterwards, a predetermined amount of hydrocarbon gas and a predetermined amount of oxidative gas are supplied to

the carburization room 17 by way of a purge line, so that an internal pressure within the carburization room 17 is allowed to be restored to its carburization pressure. Upon pressure restoration and based on the computation result obtained by processing the data representing the measured  $\text{CO}_2$  partial pressure or  $\text{CO}_2$  concentration, the carburization room 17 is allowed to control, with the use of a control line, the supply amount of at least one of the hydrocarbon gas and the oxidative gas. However, at this time, the carbon potential is set with reference to a carbon solid solubility which depends on a carburization temperature, so that such a carbon potential will be within a predetermined range so as not to produce soot.

After having performed the carburization treatment for a predetermined time period, the supply of the hydrocarbon gas as well as the oxidative gas to the carburization room 17 is stopped, and the atmosphere within the carburization room 17 is discharged so as to have the steel material kept under a reduced pressure, thereby adjusting the carbon concentration on the surface of the steel material. Then, the temperature within the carburization room 17 is lowered to the quenching temperature, and the partition door 21a is opened. Further, the partition door 21c located between the transportation room 16 and the quenching room 19 is opened, so that the steel material is transferred, under a reduced pressure, to the quenching room 19 by way of the transportation room 16, thereby performing an oil quenching treatment. After the quenching treatment, the steel material is taken out of the treatment system by way of the outlet door 20. At this moment, an adjustment of the carbon concentration on the surface of the steel material is allowed to be performed, and at the same time a control of the quenching temperature is carried out.

Furthermore, in the case of a high temperature carburization treatment ( $1050^\circ \text{C}$ ) which requires an adjustment of crystal particles, after an adjustment has been performed on the carbon concentration on the surface of the treated steel material, the steel material is transported to the gas cooling room 18 by way of the transportation room 16 as well as the partition door 21b. Then, after the pressure has been restored to a predetermined value (for example, 100 kPa) by means of  $\text{N}_2$  gas, the steel material is cooled and the  $\text{N}_2$  gas is discharged, so that the pressure over the steel material is reduced to 1 kPa or lower. In this way, under a reduced pressure and by way of the transportation room 16, the steel material is returned to the carburization room 17 so as to be heated again to a temperature suitable for a reheating treatment. Moreover, the carburization room 17 is kept at the reheating temperature for 30 minutes. Then, the  $\text{N}_2$  gas is discharged so that the pressure within the carburization room is reduced to 1 kPa or lower. Subsequently, the steel material is transported to the quenching room 19 by way of the transportation room 16, thereby performing an oil quenching treatment. In this way, after the quenching treatment has been finished, the steel material is taken out of the treatment system by way of the outlet door 20.

In fact, the inventors of the present invention have conducted the carburization treatment using the method of the present invention, with an actual process and results thereof being discussed in the following.

## EXAMPLE 1

Sections of steel material SCM 420 in the form of test pieces each having a diameter of 20 mm and a length of 40 mm were disposed at nine positions (upper and lower corner portions as well as in the central area) within the carburization room 17 whose internal temperature was controlled at  $950^\circ \text{C}$ . and whose internal pressure was controlled at 0.1 kPa or

lower. Then, the pressure within the carburization room 17 was restored to 100 kPa by charging the room with  $\text{N}_2$  gas, while the internal temperature thereof was kept at  $950^\circ \text{C}$ .

After the carburization room 17 had been kept under the above-described conditions for 30 minutes, its internal pressure was reduced to 0.1 kPa by virtue of gas discharge. Subsequently,  $\text{C}_3\text{H}_8$  gas and  $\text{CO}_2$  gas were supplied into the carburization room 17, each at a flow rate of 3.5 L/min so as to increase the internal pressure to 1.7 kPa.

Next, with the internal pressure of the carburization room 17 kept at 1.7 kPa, the amount of  $\text{C}_3\text{H}_8$  gas and/or  $\text{CO}_2$  gas being supplied to the carburization room was changed so as to control the carbon potential to 1.25%. Then, the interior of the carburization room 17 was kept at  $950^\circ \text{C}$ . for 57 minutes.

Subsequently, the supply of  $\text{C}_3\text{H}_8$  gas and/or  $\text{CO}_2$  gas was stopped and the internal pressure within the carburization room 17 was reduced to 0.1 kPa by virtue of gas discharge. Then, this internal pressure was kept for 37 minutes, while the internal temperature of the carburization room 17 was lowered to  $870^\circ \text{C}$ . during a subsequent time period of 30 minutes. Then, the steel material was transported to the quenching room 19 by way of the transportation room 16, thereby starting the oil quenching treatment.

The average carbon concentration distribution of the steel material treated in this example is shown in FIG. 3. In fact, the carbon concentrations shown in this graph represent the average values of the carbon concentrations of the steel material pieces located at the aforementioned nine positions. As a result, an effective carburization depth (0.36% C) could be found to be 0.7 mm, which was an appropriate value. Further, a photograph representing the surface organization of the treated steel material is shown in FIG. 4. It is to be noted that there were no abnormal layers formed on the surface of the steel material treated in the above described process.

When a carburization lead time of the carburization treatment in Example 1 was compared with a carburization lead time of the gas carburization treatment (which is a conventional process) using an endothermic gas, it was found that the conventional gas carburization treatment using an endothermic gas needed 118 minutes as its carburization lead time, while the carburization lead time of the carburization treatment in Example 1 was only 94 minutes, thus making it possible to shorten the carburization lead time by about 20%. In this way, using the carburization treatment method actually carried out in Example 1, it becomes possible to obtain a carburized layer having a desired depth using a shorter time period than required by the above described conventional gas carburization treatment (which requires the use of an endothermic gas). Therefore, the total energy consumption can be reduced and thus the desired economic advantage can be achieved. Moreover, since there is no soot being generated, the pieces of steel material can be placed at any position within the furnace without any limitation. In addition, the use of the present invention makes it possible to obtain carburized layers which are relatively uniform and differ little from each other in their physical and chemical properties.

## EXAMPLE 2

Example 2 is used to explain how a high temperature carburization can be carried out. Namely, sections of steel material pieces which were identical to those used in Example 1 were disposed at nine positions within the carburization room 17 whose internal temperature was controlled at  $1050^\circ \text{C}$ . and whose internal pressure was controlled at 0.1 kPa or lower. Then, the pressure within the carburization

room 17 was restored to 100 kPa by charging the room with N<sub>2</sub> gas, while the internal temperature thereof was kept at 1050° C.

After the carburization room 17 had been kept under the above-described conditions for 30 minutes, its internal pressure was reduced to 0.1 kPa by virtue of gas discharge. Subsequently, C<sub>3</sub>H<sub>8</sub> gas and CO<sub>2</sub> gas were supplied into the carburization room 17 at a flow rate of 14 L/min so as to increase the internal pressure to 1.7 kPa.

Next, with the internal pressure of the carburization room 17 kept at 1.7 kPa, the supply amount of CO<sub>2</sub> gas was controlled at a constant flow rate of 10 L/min, while the supply amount of C<sub>3</sub>H<sub>8</sub> gas was changed so as to have the carbon potential controlled at 1.4%. Then, the interior of the carburization room 17 was kept at 1050° C. for 16 minutes.

Subsequently, the supply of C<sub>3</sub>H<sub>8</sub> gas and CO<sub>2</sub> gas was stopped and the internal pressure within the carburization room 17 was reduced to 0.1 kPa by virtue of gas discharge. This internal pressure was kept for 16 minutes. Afterwards, the steel material was cooled and then heated again so as to adjust the size of the crystal particles.

In more detail, the steel material was transported from the carburization room 17 to the gas cooling room 18 by way of the transportation room 16. Then, the interior of the gas cooling room 18 was restored to 100 kPa by charging the room with N<sub>2</sub> gas, followed by cooling the same for 15 minutes. Afterwards, the N<sub>2</sub> gas was discharged and the internal pressure within the gas cooling room 18 was reduced to 0.1 kPa or lower. At this time, the steel material was transported into the carburization room 17 by way of the transportation room 16. Then, the steel material was heated so as to increase its temperature, with the heating process being conducted under a condition in which the N<sub>2</sub> gas was still present and the internal pressure within the carburization room was 100 kPa. After this condition had been kept for 30 minutes, the internal pressure within the carburization room 17 was reduced to 0.1 kPa by virtue of gas discharge, while the steel material was transported to the quenching room 19 by way of the transportation room 16, thereby starting the oil quenching treatment.

The average carbon concentration distribution of the steel material treated in this example is shown in FIG. 5. In fact, similar to the above example shown in FIG. 3, the carbon concentrations shown in this graph represent the average values of the carbon concentrations of the steel material pieces located at the aforementioned nine positions. As a result, an effective carburization depth (0.36% C) was found to be 0.73 mm, which was an appropriate value. Further, a photograph indicating the surface organization of the treated steel material is shown in FIG. 6. It is to be noted that there were no abnormal layers formed on the surface of the steel material treated in the above described process. In addition, one example of a crystal particle photograph is shown in FIG. 7. Here, the crystal particle size was #9, which was an appropriate value.

In this way, since the treatment temperature was set at 1050° C, which is a high temperature, and since the carbon potential was set at 1.4%, the carburization lead time of the carburization treatment in Example 2 could be greatly reduced. In fact, the carburization lead time in this example was reduced by about 73% compared with the aforementioned conventional gas carburization treatment (which uses an endothermic gas). Accordingly, using the carburization treatment method actually carried out in Example 2, it becomes possible to obtain a carburized layer having a desired depth, using a reduced time period than that required by the above described conventional gas carburization treatment (which uses an endothermic gas). Therefore, it is pos-

sible to reduce the total energy consumption. Moreover, since there is no soot being generated, the pieces of steel material can be placed at any position within the furnace without any limitation. In this way, the use of the present invention makes it possible to obtain carburized layers which are relatively uniform and differ little from each other in their physical and chemical properties.

### EXAMPLE 3

Example 3 was conducted based on Example 1 but using a different carburization pressure from that used in Example 1. Namely, sections of steel material pieces which were identical to those used in Example 1 were disposed at nine positions within the carburization room 17 whose internal temperature was controlled at 950° C. and whose internal pressure was controlled at 0.1 kPa or lower. Then, the pressure within the carburization room 17 was restored to 100 kPa by charging the room with N<sub>2</sub> gas, while the internal temperature thereof was kept at 950° C.

After the carburization room 17 had been kept under the above described conditions for 30 minutes, its internal pressure was reduced to 0.1 kPa by virtue of gas discharge. Subsequently, C<sub>3</sub>H<sub>8</sub> gas and CO<sub>2</sub> gas were supplied into the carburization room 17, each at a flow rate of 15 L/min so as to increase the internal pressure to 100 kPa.

Next, with the internal pressure of the carburization room 17 kept at 100 kPa, the supply amount of CO<sub>2</sub> gas and/or the supply amount of C<sub>3</sub>H<sub>8</sub> gas were changed so as to have the carbon potential controlled at 1.25%. Then, the interior of the carburization room 17 was kept at 950° C. for 57 minutes.

Subsequently, the supply of C<sub>3</sub>H<sub>8</sub> gas and CO<sub>2</sub> gas was stopped and the internal pressure within the carburization room 17 was reduced to 0.1 kPa by virtue of gas discharge. Then, this internal pressure was kept for 37 minutes, while the internal temperature of the carburization room 17 was lowered to 870° C. during a subsequent time period of 30 minutes. Afterwards, the steel material was transported to the quenching room 19 by way of the transportation room 16, hence starting the oil quenching treatment.

As a result, an effective carburization depth (0.36% C) of the treated steel material in this example was found to be 0.72 mm, which was an appropriate value, and no soot was generated.

What is claimed is:

1. A carburization treatment method comprising:  
introducing steel material into a transportation room,  
wherein the transportation room is configured to transport the steel material between a carburization room, an oil quenching room, and a gas cooling room;  
reducing the pressure in the transportation room to 0.1 kPa or lower;  
transporting the steel material after the pressure of the transportation room has been reduced from the transportation room to the carburization room by way of opening a first partition door located between the transportation room and the carburization room;  
elevating a pressure in the carburization room by introducing N<sub>2</sub> gas therein and elevating a temperature in the carburization room after the first partition door is closed;  
reducing the pressure in the carburization room to 0.1 kPa or lower by discharging the N<sub>2</sub> gas;  
supplying a predetermined amount of hydrocarbon gas and a predetermined amount of oxidative gas to the carburization room so that the internal pressure of the carburization room is 0.1 to 101 kPa, the hydrocarbon gas

being at least one of gases selected from the group consisting of C<sub>3</sub>H<sub>8</sub>, C<sub>3</sub>H<sub>6</sub>, C<sub>4</sub>H<sub>10</sub>, C<sub>2</sub>H<sub>2</sub>, C<sub>2</sub>H<sub>4</sub>, C<sub>2</sub>H<sub>6</sub> and CH<sub>4</sub>;

controlling the amount of hydrocarbon gas and the amount of oxidative gas in the carburization room with the internal pressure of the carburization room kept at 0.1 to 101 kPa such that an atmosphere within the carburization room has a high carbon potential which is slightly below a carbon solid solubility limit;

stopping the supply of hydrocarbon gas and oxidative gas and reducing the pressure in the carburization room; and after a predetermined amount of time, lowering the temperature in the carburization room to an oil quenching temperature and opening the first partition door;

transporting the steel material to the oil quenching room from the carburization room, via the transportation room by opening a second partition door located between the transportation room and the oil quenching room; and performing an oil quenching treatment on the steel material in the oil quenching room.

2. The carburization treatment method according to claim 1, wherein the atmosphere having a high carbon potential slightly below the carbon solid solubility is maintained by directly supplying at least one of the hydrocarbon gas and the oxidative gas into the carburization room.

3. The carburization treatment method according to claim 2, wherein the oxidative gas is O<sub>2</sub> gas or CO<sub>2</sub> gas.
4. The carburization treatment method according to claim 2, wherein the amount of at least one of the hydrocarbon gas and the oxidative gas being supplied to the carburization room for maintaining the atmosphere having a high carbon potential slightly below the carbon solid solubility is controlled by carrying out at least one of the following measurements: measurement of CO gas partial pressure, measurement of CO<sub>2</sub> gas concentration, measurement of CO<sub>2</sub> gas partial pressure measurement of CO<sub>2</sub> gas concentration, measurement of O<sub>2</sub> gas concentration, measurement of H<sub>2</sub> gas partial pressure, measurement of H<sub>2</sub> gas concentration, measurement of CH<sub>4</sub> gas partial pressure, measurement of CH<sub>4</sub> gas concentration, measurement of H<sub>2</sub>O partial pressure, measurement of H<sub>2</sub>O concentration, and measurement of dew point, all within the carburization room.
5. The carburization treatment method according to claim 1, comprising, after the oil quenching, removing the steel material through an outlet door.
6. The carburization treatment method according to claim 5, comprising transporting the steel material to the gas cooling room from the carburization room, via the transportation room, by opening a third partition door located between the gas cooling room and the transportation room.

\* \* \* \* \*